

A. M. FAIRCHILD.

SPARK PLUG.

APPLICATION FILED MAY 27, 1918.

1,369,274.

Patented Feb. 22, 1921.



Witness,  
S. S. Mann,

Inventor,  
Alice Maude Fairchild.

# UNITED STATES PATENT OFFICE.

ALICE MAUDE FAIRCHILD, OF CHICAGO, ILLINOIS, ASSIGNOR TO CHARLES K. HARDING, OF CHICAGO, ILLINOIS.

## SPARK-PLUG.

1,369,274.

Specification of Letters Patent. Patented Feb. 22, 1921.

Application filed May 27, 1918. Serial No. 236,933.

*To all whom it may concern:*

Be it known that I, ALICE MAUDE FAIRCHILD, a citizen of the United States, and a resident of the city of Chicago, in the 5 county of Cook and State of Illinois, have made certain new and useful Improvements in Spark-Plugs, of which the following specification is such a full, clear, and exact description as will enable others skilled in 10 this art and the other arts to which this art most nearly appertains to make and use the same.

The accompanying drawings show a spark plug illustrative of the type of apparatus 15 which forms the subject of my invention.

My invention relates generally to electrical ignition devices for internal combustion engines and more particularly to the detachable portion forming part of the wall 20 of the inclosed space within which the explosion of the fuel mixture is produced by the discharge of a high tension current across the arc formed between the terminals of a plurality of conducting electrodes.

25 This detachable portion 1 commonly called a spark plug usually carries two metallic terminals 2 and 3 with one of the conducting metallic electrodes extending entirely therethrough and a non-metallic insulating means 4 forming a portion of the wall and extending entirely therethrough from the inside to the outside of the combustion space.

Figure 1 is the vertical section view 35 through this improved spark plug, and

Fig. 2 is the vertical section through the insulator.

The conducting electrode extending through the plug as well as the conducting 40 parts connecting with the opposite terminal may be made of any suitable metallic substance as most of the metals now commonly used in spark plugs have sufficient mechanical strength and electrical conductivity.

45 One of the objects of my invention is to improve spark plugs by the employment of certain oxids in the construction of the non-metallic insulating means. I have found that zirconium oxide and zirconium silicate 50 when constituting from 50 to 90% of the mass forms a ceramic structure having properties which produce an insulating non-metallic structure that has more suitable physi-

cal characteristics and desirable properties than any other of the ceramic materials such as stoneware, china and porcelain heretofore known or used in spark plugs.

Zirconia ( $ZrO_2$ ) zirconium oxide has been well known for many years having been used largely in incandescent mantles of the 60 early Welsbach type and their immediate predecessors. It was next largely used as a substitute for the lime structure in oxyhydrogen or calcium light and its fire resisting properties are well known.

65 The fact that zirconia formed an important constituent in the structure of the glower in the Nernst lamp might lead to the assumption that it would be unsuitable for use as a heat resisting insulating structure 70 for spark plugs but I have found by numerous tests within the last two years that it forms a more desirable constituent of a body for a spark plug insulator than any other of the numerous oxids of other compounds with which I have experimented and that it can be substituted with great improvement for china clay, feldspar, silica, 75 magnesium silicate and other constituents heretofore employed in stoneware, china or porcelain insulators.

Of the various processes for forming earthen ware structures those depending on water shrinkage such as forming on a wheel or shaping in a plaster Paris mold or casting a thin slip can not be employed where large quantities of zirconia is used on account of its lack of the properties characteristic of clay, that is, capillary shrinkage 80 into a hard compact mass but structures containing a large quantity of finely ground zirconium silicate such as the mineral zircon or finely ground baddeleyite a natural ore containing a high percentage of zirconium oxide with from 5 to 15% plastic clay can be 95 readily formed into quite intricate shapes by what is known as the dry forming process frequently described as pressing a moist dust into steel molds.

A moist granulated zirconium mass containing as little as 5% of clay and about 12% of water can be placed in a closely fitting steel die and subjected to a pressure of from 5 to 8,000 pounds to the square inch and formed into a structure that will shrink 105 very little in air drying or oven drying and

which may be fired to any high temperature available without danger of undue fusing or shrinkage.

Having now fully described my invention 5 what I claim is:—

1. A spark plug having metallic conducting electrodes and non-metallic wall forming and insulating means consisting of a ceramic structure formed from plastic clay 10 and zirconium compounds.

2. A spark plug having metallic conducting electrodes and non-metallic wall forming and insulating means comprising a ceramic structure consisting of zirconia 15 compounds and a clay binder.

3. A spark plug having metallic conducting electrodes and non-metallic wall forming an insulating means consisting of a ceramic structure containing clay and zirconium compounds.

4. As a new article manufactured, an insulator for spark plugs comprising a ceramic structure of clay containing zirconia compounds in varying proportions.

In testimony whereof I have signed this 25 specification at Chicago, in the county of Cook and State of Illinois, this 29 day of May, 1917.

ALICE MAUDE FAIRCHILD.